

Feb. 1, 1938.

J. H. DE BOER ET AL

2,106,868

METHOD OF OBTAINING PHOTOGRAPHIC CONTRASTS

Filed Dec. 19, 1934

Formation speed of the Coloring Matter

Fig. 1.



Increasing Alkalinity and decreasing Acidity

Intensity of the final Color

Fig. 2.



Quantity of Light Actinically Active

Inventors

Jan Hendrik De Boer  
and Klaas Hinderikus Klaassens

By

*Elle B. De Boer*  
Attorney.

## UNITED STATES PATENT OFFICE

2,106,868

## METHOD OF OBTAINING PHOTOGRAPHIC CONTRASTS

Jan Hendrik de Boer and Klaas Hinderikus  
 Klaassens, Eindhoven, Netherlands, assignors  
 to N. V. Philips' Gloeilampenfabrieken, Eindhoven, Netherlands

Application December 19, 1934, Serial No. 756,832  
 In Germany December 27, 1933

6 Claims. (Cl. 95—6)

This invention relates to a method of obtaining photographic contrasts with the aid of light, and more particularly to obtaining contrasts on a layer which has been sensitized by means of a naphthalene diazonium compound.

According to our invention, the formation of photographic contrasts is obtained by means of an actinic exposure of a self-developing layer sensitized by means of a naphthalene diazonium compound.

In the U. S. patent application Ser. No. 612,364 of De Boer, Dippel and Alink, now Patent No. 2,034,508 there has been described a process using a "self-developing" light-sensitive material formed of a benzene diazonium compound, which diazonium compound during exposure to light does not form coloring matter, but partly decomposes and the decomposition products, subsequently to the exposure, form with the remaining undecomposed diazonium compounds a colored substance.

By the term "self-development", as used herein, is meant the property of forming, as a result of and subsequently to an exposure to actinic light, coloring matter by means of the union between the light decomposition product—formed from a diazonium compound in the light sensitive layer during the exposure—and the available excess of diazonium compound, without the addition of any further chemical reagents such as ammonia gas or alkaline solutions, and correspondingly a light-sensitive material having such property, is referred to as "self-developing", which promotes the obtention of a minimum moisture content of the layer.

Such a "self-developing" light-sensitive layer as photographic material has various advantages, among others that it is not subjected to after-treatments with solutions of chemical substances for development and fixation, which not only eliminates the expense and work involved in such treatment, but also avoids the risk of distortion caused by such wet treatments.

According to the present invention, instead of using benzene diazonium compounds, naphthalene diazonium compounds are used as "self-developing" materials, which compounds, under the conditions more fully to be described hereinafter, give a material of greater stability than can be obtained with the "self-developing" layer formed with benzene diazonium compounds.

It has already been suggested to use a light-sensitive layer containing the compound consisting of 1-diazonium-2-hydroxynaphthalene-4-sulfonic acid, sodium carbonate and tartar emetic for

photographic purposes. Thereby, upon exposure, coloring appears on those portions which have been exposed to light and thus negative images are obtained. The exposed material is subjected to treatment in a diluted aqueous solution of sodium carbonate. It was found that good prints can not be obtained by this process, as such washing operation causes the image to fade or disappear, not only if the solution is quite dilute, but even if only water is used.

It has also been suggested to use the above-mentioned naphthalene diazonium compound to obtain positives from positives by subjecting the material containing said compound after its exposure—during which exposure it is "copied out"—to daylight with the template removed, and subsequently developing it in alkali. In this manner a substance, which in alkaline solution unites with the non-converted diazonium compound to form a coloring matter, is produced at such points which were not exposed to light when the original "copying out" under the positive took place.

Finally it has been suggested to use the above-mentioned naphthalene diazonium compound to obtain an image without the use of subsequent chemical treatment. Thereby the light-sensitive layer was exposed under a template or tracing, and the so-exposed light-sensitive layer thereafter subjected to further exposure in daylight—with the template or tracing removed therefrom—and then left in a dark place where, and it has been suggested that after a certain time interval, upon the initially unexposed portions colored matter was automatically formed. However, it was found that with this, colour formation did not take place at all, even if the material kept in the dark for a very long time f. i. three weeks.

We have found that a close connection exists between the pH value of a layer sensitized with a naphthalene diazonium and the formation of coloring matter by self-development and that by imparting to the layer a suitable pH value, a satisfactory self-development, in that no or substantially no formation of coloring takes place during the actual exposure, can be obtained.

According to our invention, layers sensitized by naphthalene diazonium compounds and having or being in a medium having a properly selected pH value, are subjected to the exposure of actinic light under a template, after which "self-development" of the light-sensitive layer takes place.

We have furthermore found that the speed at which the formation of the coloring matter takes place, in the process under consideration, depends

upon the moisture content which the light-sensitive layer possesses, or is capable of taking up during the exposure, and that with increasing moisture content the formation speed of 5 coloring matter is increased; furthermore, that to obtain the desired results, the amount of actinic light used for the exposure, the pH value of the light-sensitive layer, and the moisture content of the layer have to be in proper relationship; this relationship depending upon the specific naphthalene diazonium compound used.

The invention will be more fully explained in connection with the following example and the drawing forming part of the specification, and 15 in which:

Figure 1 is a diagram showing the dependency of the formation speed of the coloring matter upon the pH value (acidity or alkalinity) of the light-sensitive material, and

20 Fig. 2 is a diagram showing the relation between the intensity of the final coloring obtained and the amount of actinically acting light striking the light-sensitive layer.

Referring to Figure 1, the abscissae give the 25 pH values of the light-sensitive layer, whereas the ordinates give the corresponding formation speed of the coloring matter.

30 The curve 8 represents the formation speed of the coloring matter for a given moisture content of the layer and for different pH values (acidities and alkalinites) of the light-sensitive layer.

To obtain the desired contrast effect it is required first of all, that during the exposure the 35 image be "copied out" i. e. that the diazonium compound be decomposed at the exposed portions and, that the speed of decomposition of the diazonium compound be greater, during the exposure than is the speed at which the coloring 40 matter is formed. Secondly, that after the exposure there shall be "self-developing", i. e. that coloring matter be formed by undecomposed diazonium compound entering into reaction with the decomposition products of the diazonium 45 compound.

Unless the diazonium compound is photochemically decomposed, evidently no "copying out" can take place. On the other hand, if the formation speed of the coloring matter is greater than 50 the speed of decomposition, formation of coloring matter takes place with such rapidity during the exposure, that "copying out" is impossible, even if the most intensive available light sources are used.

55 In Fig. 1, the line 10, which is parallel to the abscissa axis, represents the speed of photochemical decomposition for a given light intensity or actinic light energy falling on the light-sensitive 60 layers during the exposure. The diagram is shown to be divided, according to the pH value of the light-sensitive layer, into three zones marked A, B and C. Of these zones, zone A extends from the ordinate axis to the ordinate through point 1, the latter point falling somewhat to the right of the point 12 (which corresponds to the pH value 7 or chemical neutrality), the point 1 representing the alkalinity at which the formation speed of coloring matter is first discernible.

65 The zone B extends from the ordinate passing through point 1 to the ordinate passing through point 2, which latter point is the intersection of the curve 8 with the line 10, while the zone 70 C extends towards the right of zone B.

It should be well understood that the pH values and the formation speed of the coloring matter are not drawn to scale, and the curves 8 and 9 merely indicate the general character of the relationship without giving exact values. 5

Taking first the zone A, it will be noted that, with the pH values lying within this zone, the diazonium compound can be photochemically decomposed. However, in this zone no formation of coloring matter can take place either during 10 the actual exposure under the template, or thereafter when keeping the exposed print in the dark, and therefore the zone A is unsuitable for the purpose of the invention.

In zone C the formation speed of the coloring 15 matter is greater than is the speed of the decomposition of the diazonium compound and therefore the formation of coloring matter takes place so rapidly during the exposure that no "copying out" is possible, even by means of the 20 most intensive available light sources.

Referring now to zone B, which extends from 25 layers having slight alkalinity to layers having moderate alkalinity, it will be noted that the formation speed of the coloring matter, while increasing toward the right, remains smaller than the speed of photochemical decomposition. Thus, light-sensitive layers having pH values falling within the zone B can be "copied out" 30 and subsequently produce coloring matter by "self-development".

The zone B is, therefore, the only zone which 35 is suitable for the process of the invention and to obtain a reasonable formation speed of the coloring matter it is desirable to work in the right-hand portion of this zone, although preferably staying a reasonable distance to the left of the point 2, as too close an approach to point 2 increases the danger of coloration during the 40 exposure.

If, instead of the assumed light intensity used during exposure and corresponding to line 10, a higher intensity of exposure is used, as represented by the dot-and-dash line 13, the useful 45 zone B is extended toward the right, as indicated by the intersection point 14 of line 13 with curve 8.

As stated, the formation speed of the coloring matter also depends upon the quantity of moisture which the light-sensitive layer possesses or 50 is capable of taking up during exposure, and the formation speed decreases with decreasing moisture content and vice versa.

The dotted curve 9 represents the formation 55 speed of the coloring matter for a moisture content lower than in the case of curve 8. Thereby as appears from Fig. 1, the curve 9 and line 10 intersect at a point 2' which point lies to the right of point 2; thus the zone B is extended toward the right by using a lower moisture content. 60

From the above it will be thus noted that the zone B can be extended by using either a higher light intensity for the exposure or a lower moisture content of the light-sensitive layer. However, the extension of the useful zone B is limited by the fact that a very high alkalinity will so strongly increase the formation speed of the coloring matter as to prevent the possibility of 65 "copying out".

The importance of the proper relationship between the speed of photochemical decomposition of the diazonium compound and the formation speed of the coloring matter by "self-develop- 70

ment" will further appear from Fig. 2. In this figure curve 11 gives the intensity of the final coloring obtained as a function of the amount of actinic-light striking the light-sensitive layer during the exposure. Thereby the abscissae give the amount of actinic light and the ordinates the intensity of the resulting coloring.

In the example given, a positive is made of a tracing whereby, in the print obtained, upon actinic exposure of the light-sensitive layer, the portion corresponding to the lines of the tracing which will remain either unexposed or only slightly exposed to light, appear as colored lines, while the blank and thus transparent portions of the tracing will cause the corresponding portions of the print to be fully exposed and thus to appear uncolored. Thus a positive from a positive is obtained.

When the light-sensitive layer is exposed to light under the tracing, it is struck under the lines of the tracing by a small quantity of light represented by the point 3, to which corresponds the ordinate 15, whereas under the blank or transparent portions of the tracing the light-sensitive layer is struck by a comparatively large amount of light, represented by the point 4 whose ordinate is zero.

The "self-development" of the print may take place in the dark or by subjecting the print, after removal of the tracing, to a slightly actinic light. In this latter case an equal and small amount of light uniformly strikes all of portions of the photographic layer, this amount of light being indicated by the equal portions 3-6 and 4-5 of the abscissa axis. Thus, the total amount of actinic light which strikes the portions to be colored corresponds to the abscissa 6, whereas the total amount of actinic light which strikes the portion to remain uncolored corresponds to the abscissa 5.

It will be seen that the intensities of the final coloring are represented by the ordinate 7 corresponding to the amount of light 6, and is practically zero corresponding to the amount of light 5. It will be thus noted that at the points 4 and 5 the light intensity is so great that the entire diazonium compound becomes decomposed, and no undecomposed diazonium compound remains to form, with the decomposed diazonium compound, coloring matter.

Instead of increasing the intensity of coloring from point 15 to point 7 by means of after-exposure, this can be also achieved by moderate heating of the layer or by increasing its moisture-content.

From the above it will appear that in case a positive is to be obtained from a positive, a very definite relationship must exist between the speed of color formation and decomposition, as otherwise the desired sharp contrast effect is not obtained. The same applies, as will be later pointed out, when negatives are to be obtained from a positive.

In practice the ideal conditions represented by Fig. 2 are not always obtainable, and even on the fully exposed portions of the print a small amount of color formation may take place during the exposure.

This can be obviated and a perfectly white, i. e., uncolored background can be obtained if the sensitive carrier, for instance the paper carrying the light-sensitive substance, is subjected to intensive drying in such a manner that the paper retains a moisture content of less than 1%.

By the "degree of moisture" of the paper, as

used herein, is to be understood here to mean the percentage decrease in weight which air-dried paper experiences when it is heated for 24 hours at a temperature of 25° C. within an enclosure dried by fresh phosphorus pentoxide. For a correct understanding, it must be mentioned that drying in an enclosure kept dry by means of phosphorus pentoxide results in a greater decrease of the moisture content of the paper than the generally used method of drying according to which the paper is heated at comparatively high temperature, say from 105 to 110° C. Thus, for example, it has been found that so-called air-dry paper, when dried at a temperature up to 110° C. showed a decrease in weight of 6½%, but when dried within an enclosure kept dry by means of phosphorus pentoxide is shown a decrease in weight of 7.9%.

Such intensive drying may also be achieved by subjecting the material to a flow of moisture-free gas. Such a moisture-free gas can be obtained by drying the gas by means of a suitable drying medium such as phosphorus pentoxide. Alternatively, a gas may be freed from all its moisture by freezing out the moisture from the gas at a very low temperature.

Such intensive drying of photographic material comprising diazonium compounds is described and broadly claimed in the U. S. Patent 1,973,788 to Alink and De Boer.

The following specific example will serve to further illustrate the invention:

#### Example

The sensitized photographic material adapted for making prints from tracings is obtained by soaking a suitable paper carrier in a solution of 1% 1-diazonium-2-hydroxynaphthalene-4-sulfonic acid (1 mol.) + 0.6% anhydrous sodium carbonate in water, and by subsequently drying it in air.

To make the print the sensitized paper is exposed under a template, for instance a tracing, for a time interval of about three minutes, and using as a light source, for instance a 5 kw. incandescent filament lamp placed at a distance of about 25 cm. from the template.

Immediately after the exposure the image is faintly visible, while the background is uncolored.

The so-exposed paper is then allowed to remain in the dark during which the "self-development" takes place, which may be accelerated by the presence of water vapor. The "self-development" may also be accelerated by putting a moistened cloth heated to a temperature of about 100° C. on the paper.

By the above method a positive is obtained from a positive and the image has a brownish-yellow tone. If the quantity of anhydrous sodium carbonate is increased to 1.2%, an image of lilac-violet tone is obtained.

To obtain a completely white background, as has been stated before, the sensitized paper is subjected to intensive drying before being used for the exposure. With the moisture content thus minimized, the formation speed of the coloring matter during the exposure is so reduced that no coloring whatsoever takes place at the fully exposed portions.

Instead of using sodium carbonate other alkaline agents, especially salts giving slightly alkaline reaction, are suitable for carrying out the invention, for example, sodium borate.



or sodium phosphate ( $Na_3PO_4 \cdot 10H_2O$ ), or sodium selenite ( $Na_2SeO_3$ ), which in proper amounts, which of course depends upon their alkaline reaction, will give the light-sensitive layer the desired pH value.

For example for 1 mol. diazonium compound  $3\frac{1}{2}\% Na_2B_4O_7 \cdot 10H_2O$  or 6%  $Na_3PO_4 \cdot 10H_2O$  or 4%  $Na_2SeO_3$  may be used.

It is also possible to obtain by means of the invention negatives from a positive. For this purpose the time of exposure under the template is made extremely short, so that the portions of the print which fall under the transparent portions of the template receive an amount of light corresponding to less than 6 (Fig. 2), whereas the amount of light energy falling on the positions of the point under the dark portions of the template will be considerably less and practically zero. The so-exposed print is then subjected to 20 "self-development" in the dark in the presence of air.

As will appear from Fig. 2, the "exposed" portions of the print will be now strongly colored, whereas the "unexposed" portions will remain 25 substantially colorless.

However, to insure that the available non-decomposed naphthalene diazonium compound remaining at the "non-exposed" portions of the print does not, by gradual decomposition, cause 30 darkening of the unexposed portions, after the "self-developed" negative print is removed from the dark, they are rapidly and completely decomposed by a fixation process, consisting in subjecting the print to strongly actinic light without a template, whereby a complete decomposition takes place at the previously "unexposed" 35 portions, and so rapidly as to prevent any color formation on these portions.

While we have described our invention in connection with specific examples and in specific 40 applications, we do not wish to be limited thereto, but desire the appended claims to be construed as broadly as permissible in view of the prior art.

What we claim is:

45 1. In the method of producing photographic contrasts by selectively exposing to actinic light a layer sensitized with a naphthalene diazonium compound and forming coloring matter by the union of the diazonium compound and its light-decomposition product, the step of imparting to said layer prior to exposure a pH value lying within a range having an upper limit corresponding to the point at which there will be substantially no formation of coloring matter during the exposure and a lower limit greater than 7 and corresponding to the point at which the color formation subsequent to the exposure can be obtained solely by the influence of water and without the addition and removal of any chemical substance.

50 2. In the production of photographic contrasts by selectively exposing to actinic light a layer sensitized with a naphthalene diazonium compound to partially decompose the compound at selected portions and by forming coloring matter by the union of the compound and its light-decomposition product, the steps of alkalinizing the layer prior to exposure to impart thereto a pH value lying within a range having an upper limit corresponding to the point at which there will be substantially no formation of coloring matter during the exposure and a lower limit greater than 7 and corresponding to the point at which subsequent color formation can be ob-

tained solely by the influence of water, and exposing the layer without the formation of pronounced coloring matter.

5 3. In the method of producing photographic contrasts by selectively exposing to actinic light a layer sensitized with a naphthalene diazonium compound and forming coloring matter by the union of the diazonium compound and its light-decomposition product, the step of adding an alkaline-reacting salt to said layer to impart thereto a pH value lying within a range having an upper limit corresponding to the point at which there will be substantially no formation of coloring matter during the exposure and a lower limit greater than 7 and corresponding to 15 the point at which the color formation can be obtained subsequent to the exposure solely by the influence of water and without the addition or removal of any chemical substance.

4. In the method of producing photographic 20 contrasts by selectively exposing to actinic light a layer sensitized with a naphthalene diazonium compound and by forming coloring matter by the union of the diazonium compound and its light-decomposition product, the steps of imparting to 25 said layer prior to the exposure a pH value lying within a range having an upper limit corresponding to the point at which there will be substantially no formation of coloring matter during exposure and a lower limit greater than 7 30 and corresponding to the point at which the color formation can be obtained solely by the influence of water and without the addition or removal of any chemical substance, and drying the layer prior to exposure to reduce its moisture 35 content to below 1%.

5. The method of producing photographic prints, comprising the steps sensitizing a layer with a naphthalene diazonium compound, alkalinizing the layer to give same a pH value less 40 than that value at which there will be substantially no formation of coloring matter during the exposure and more than that value at which the color formation can be obtained solely by the influence of water and without the addition or removal of any chemical substance, drying the 45 layer to reduce its moisture content to below 1%, selectively exposing the layer to actinic light to partially decompose the diazonium compound on selected portions without the formation of appreciable coloring matter, and wet-ironing the exposed layer at a temperature of about 100° C. to form coloring matter at the selected portions by the union of the diazonium compound and its light-decomposition product.

55 6. In producing photographic contrasts by selectively exposing to actinic light a layer sensitized with a naphthalene diazonium compound and forming contrasts by the union of the diazonium compound and its light-decomposition 60 product, the steps of alkalinizing the unexposed layer to a degree of alkalinity lying within a zone having an upper limit corresponding to the point above which there will be appreciable formation of coloring matter during the exposure and a 65 lower limit corresponding to the point above which color formation can be obtained subsequent to the exposure solely by the influence of water and without the addition or removal of any chemical substance, and selectively exposing the 70 layer to partially decompose the compound at selected portions without the formation of appreciable coloring matter during the exposure.

JAN HENDRIK DE BOER.

KLAAS HINDERIKUS KLAASSENS. 75

CERTIFICATE OF CORRECTION.

Patent No. 2,106,868.

February 1, 1938.

JAN HENDRIK de BOER, ET AL.

It is hereby certified that error appears in the printed specification of the above numbered patent requiring correction as follows: Page 1, second column, line 43, after the word and comma "self-development," insert limited; and that the said Letters Patent should be read with this correction therein that the same may conform to the record of the case in the Patent Office.

Signed and sealed this 15th day of March, A. D. 1938.

(Seal)

Henry Van Arsdale,  
Acting Commissioner of Patents.